

July 21, 1931.

H. L. COLES

1,815,186

METHOD OF CASTING METALS

Original Filed Feb. 20, 1929

*Fig. 1.*



*Fig. 2.*



*Fig. 3.*



## UNITED STATES PATENT OFFICE

HENRY L. COLES, OF HAMILTON, OHIO, ASSIGNOR TO GUARDIAN METALS COMPANY, OF HAMILTON, OHIO, A CORPORATION OF DELAWARE

## METHOD OF CASTING METALS

Application filed February 20, 1929, Serial No. 341,381. Renewed January 12, 1931.

This invention relates to metal founding, and more particularly to an improved method of producing shrinkless castings of metals or alloys having a relatively high coefficient of expansion.

As is well known, molten metals decrease in volume on cooling, the shrinking of such metals in a mold after casting, causing grave inconveniences due to the surfaces of the cast body being considerably depressed and the corners rounded or shrunken. To prepare such castings in a condition for use, it is necessary to chip out the shrunken faces and replenish the missing metal with fresh, molten metal. This latter procedure is not only costly, involving considerable expense in both time and labor, but the results are not uniform, and the process may have to be repeated in order to secure passable castings.

The deficiencies met with in the practice of metal founding, are marked in ferrous castings, and even more in non-ferrous castings. This is due to the fact that the non-ferrous metals which are commonly used, such as copper and its alloys, have a higher shrinkage coefficient than iron and its alloys. As an example of this, it is noted that copper has a shrinkage coefficient of substantially 1.42 percent, which is roughly about 0.25 inch per foot.

It is an object of this invention to provide an improved casting process for preventing the formation of shrink holes, or depressions, or the like.

Yet another object of this invention is the provision of an improved means for securing shrinkless castings.

These and other desirable objects and advantages of the present invention will be described in the accompanying specification and illustrated in the drawings, a preferred embodiment being given by way of illustration only, for since the underlying principles may be applied to other specific processes, it is not intended to be limited to the one herein shown, except as such limitations are clearly imposed by the appended claims.

Fig. 1 represents a vertical cross section 50 of a bottom pour mold, showing the applica-

tion of the principles of the present invention.

Fig. 2 is a view similar to Fig. 1 showing the application of the present invention to the top pour mold, and Fig. 3 is a vertical cross section of an ingot showing the difficulties usually encountered in ordinary casting.

In the practice of the invention, a mold of suitable form is provided, preferably of the bottom pour type. This structure may comprise a bottom portion or drag 1, having sides 2 and floor 3, with or without a bottom pouring gate 4, the construction of which is well known to those skilled in the art. The drag is rammed up in the usual manner with molding sand or any other suitable material, indicated generally at 5, and the pattern withdrawn, after the cope 6, prepared in the same manner, is finished. Suitable luting 7, 70 may be provided between the cope and drag. The materials used and their manner of application are well known to those skilled in the art and need no further explanation here.

As has been stated hereinbefore, the major difficulty met with in casting metals to form, is the shrinkage resulting from the cooling of the metal, with a resulting deformation of the surfaces of the casting. This difficulty has now been overcome by the discovery that the initially chilled skin of the casting may be held in place by providing suitable supports 8 in the cope or walls. These members may be of any suitable dimensions, and preferably are of sufficient length to protrude through the cope and walls and into the casting chamber 9, for a considerable distance.

As the molten metal rises through the gate 4 and into chamber 9, it contacts with the members 8, and progressively melts them, the upper skin of the advancing metal being contacted with and supported by their unmelted portions. These members 8, are embedded in the cope or walls for a sufficient distance, usually the entire thickness, to enable them to support the weight of the chilled skin, indicated generally at 10, thus permitting the volume of the metal in the body of the cast-

75

85

90

95

100

ing to remain constant during cooling, due to the replenishment of the shrinkage metal by other metal supplied through gate 4.

It will, of course, be understood that gate 4, is suitably connected to a reservoir of molten metal so disposed and arranged as to provide a sufficient head for replacement metal to maintain the body of the casting at its maximum volume during cooling, and 10 prevent the shrinkage of the surfaces.

The combination of the surface support for the skin of the casting by the supporting members 8, and the maintenance of maximum casting volume by providing a sufficient excess of metal to take care of shrinkage, gives highly novel and satisfactory results. Constant use of the process daily for substantially a year shows no trouble due to the necessity of filling shrink holes and the 20 like, as has been required heretofore.

While the support members have been shown as inserted and anchored in the cope, it will be understood that additional such members may be disposed in the walls of the 25 drag, without departing from the spirit and scope of the invention. Such procedure will be particularly suited for use in the making of massive castings, such as are used in safes, vault walls, and other massive 30 constructions.

Referring now to Fig. 2, there is shown a conventional mold set up, comprising a cope 12, and drag 13, with mold sand 14, which has been rammed in place to form a mold 35 suitable for casting. The mold is gated at 15 in the usual manner, and in addition, rods 16, of any suitable material and shape, are inserted through the molding sand into the molding space 17, in the manner previously 40 described. The fundamental features involved here are exactly the same as those previously described, and no further discussion is necessary.

As illustrating the difficulties overcome by 45 the practice of the present invention, there has been shown in Fig. 3 a diagrammatical example of a solid ingot which has been cast according to ordinary foundry practice. It will be noted that the body of the casting 17, 50 has shrunken corners 18, and a very much shrunken face 19. As has already been intimated, in order to prepare such castings for use, it has been necessary to chip out the shrunken face of the casting and add sufficient new metal 20, to replace that lost by shrinkage and the subsequent chipping operations.

It is also to be noted that, in order to 55 secure true plane surfaces on the several faces of the ingot itself, it is necessary to machine them, a condition which is avoided by the principles of my invention wherein the several faces are held in absolute contact with 60 the surfaces of the mold by reason of the re-

taining rods and the weight of metal in the risers and gates of the molds.

The advantageous features of the present invention may be applied to small castings of any size and shape without departing from the fundamental principles herein set forth. In such instances the size of the supporting members may be varied to suit, and the pouring gate positioned in the cope, in the ordinary manner. 70

As intimated above, the present invention is adapted for use with a wide variety of metals, and while the preferred embodiment herein disclosed refers more particularly to copper and its alloys, the members 8 preferably being of trolley wire size, or the like, the use of any and all metals is comprehended. The members 8 may be made of any suitable metal, usually the same as that of the metal used for casting. 75

It will now be seen that there has been provided an improved process and means for preventing shrinkage in metal castings, which are adapted for use with all kinds of metals, and more particularly for use with 80 massive castings of the type described.

What is claimed is:

1. The improvement in the art of casting metals which includes supporting a semi-molten body of metal from the walls of a 95 mold.

2. The improvement in the art of casting metals which includes supporting a semi-molten body of metal from the walls of a mold, whereby to prevent shrinkage of the 100 metal on cooling.

3. The improvement in the art of casting metals which includes supporting a semi-molten body of metal from the walls of a mold, and maintaining a pressure on the body 105 of the metal sufficient to compensate for normal shrinkage losses.

4. The improvement in the art of casting metals which includes supporting a semi-molten body of metal from the walls of a 110 mold, and maintaining a sufficient head of metal on the said molten body to compensate for shrinkage on cooling.

5. The improvement in the art of casting metals which includes supporting a semi-molten body of metal from the cope of a 115 mold.

6. The improvement in the art of casting metals which includes supporting a semi-molten body of metal from the cope of a 120 mold, whereby to prevent shrinkage of the metal on cooling.

7. The improvement in the art of casting metals which includes supporting a semi-molten body of metal from the cope of a 125 mold, and maintaining a pressure on the body of the metal sufficient to compensate for normal shrinkage losses.

8. The improvement in the art of casting metals which includes supporting a semi- 130

- molten body of metal from the cope of a mold, and maintaining a sufficient head of metal on the said molten body whereby to compensate for shrinkage on cooling.
8. A support for cast metal masses, including a plurality of metal members embedded in the walls of a mold and projecting an appreciable distance therein.
10. A support for cast metal masses, including a plurality of metal rods embedded in the walls of a mold and projecting an appreciable distance therein.
11. A support for cast metal masses, including a plurality of metal members embedded in the cope of a mold and projecting an appreciable distance into the mold chamber.
12. A support for cast metal masses, including a plurality of metal rods embedded in the cope of a mold and projecting an appreciable distance into the mold chamber.
13. A support for copper castings, including a plurality of copper members embedded in the walls of a mold and projecting an appreciable distance into the mold chamber.
14. A support for copper castings, including a plurality of copper rods embedded in the walls of a mold and projecting an appreciable distance into the mold chamber.
15. In a metal casting mold of the type described, in combination, a mold having top, bottom and side walls, suitable gates for the admission of molten metal into the chamber formed by the said walls, and means embedded in the walls and projecting into the chamber, said means being adapted to support the skin of the molten mass and be progressively melted to an extent by the advancing metal.
16. In a metal casting mold of the type described, in combination, a mold having a cope and drag together with suitable gates for the admission of molten metal to the mold, means embedded in the cope and projecting into the mold chamber, said means being adapted to support the upper skin of the molten mass and be progressively melted to an extent by the advancing metal, and means adapted to replenish the diminution of the metal of the mold normally caused by shrinkage on cooling.

This specification signed this 11 day of Feb., 1929.

HENRY L. COLES.